

Nov. 8, 1932.

T. H. DOWLEN

**1,886,380**

## METHOD OF OXIDIZING ASPHALTIC OILS

Filed Oct. 30, 1929



## UNITED STATES PATENT OFFICE

TOM H. DOWLEN, OF LOS ANGELES, CALIFORNIA, ASSIGNOR TO RICHFIELD OIL COMPANY OF CALIFORNIA, OF LOS ANGELES, CALIFORNIA, A CORPORATION OF DELAWARE

## METHOD OF OXIDIZING ASPHALTIC OILS

Application filed October 30, 1929. Serial No. 403,644.

This invention relates to a method of processing asphaltic oils for the manufacture of oxidized asphaltic products, which may be employed as cementing agents for roofing material, battery sealing compounds and like purposes, where a flexible asphaltic cementing agent is required with a relatively high melting point.

This application is an improvement on the processes known in the art where asphaltic oils are agitated with air at oxidizing temperatures, in that a more uniformly regulated temperature can be maintained without liability of overheating the asphaltic oil under treatment.

In the conventional method of oxidizing asphaltic oils, for the production of oxidized asphalt, air or air and steam is introduced into a cylindrical still containing the asphaltic oil through spray lines and at the same time the asphaltic oil or petroleum oil residuum contained in the still is heated to a temperature sufficient to obtain an oxidizing reaction, which may range from approximately 400 to 550 degrees F. or higher; or asphaltic oil, which may be any petroleum oil, and may contain varying percentages of paraffin wax, may be passed once through a heating coil, commingled with air, or air and steam, to heat the same to an oxidizing temperature and then through a container or still for completing the oxidizing reaction. By such methods, a uniform product cannot be obtained, since a uniform temperature cannot be maintained due to the oxidizing reaction which is exothermic. The added exothermic heat frequently overheats the asphaltic oil to a point of cracking or other decomposition reactions, thereby rendering the product more brittle or less ductile than it would be if a uniform oxidation had been effected at a definite temperature.

Also by the well-known batch still method, the time required to convert a batch of asphaltic oil into an oxidized product suitable for the manufacture of roofing felt requires approximately 24 hours, while by my invention the reaction is accomplished in about one-half that time.

Now, I have discovered an improvement

in the art of oxidizing petroleum oils in which the difficulties and various disadvantages before mentioned may be overcome by a continuous method of oxidizing the petroleum oil in stages with air while passing through a plurality of containers, each container being provided with a plurality of connected compartments, separating the residual air and volatile products of the oxidizing reaction from the oil and continuously extracting the exothermic heat produced by the said oxidation, thereby producing an oxidized product which is more suitable for cementing agents.

Briefly stated, the invention comprises passing petroleum oil residuum at a uniform oxidizing temperature continuously through a container provided with a plurality of connected compartments, separately introducing an individual supply of air into each compartment of said container, separating the residual air and volatile products of the oxidizing reaction from each compartment, passing the oil, from which the residual air and volatile products of the reaction have been separated, through a cooling coil provided with cooling means to extract the heat of the oxidizing reaction; passing the oil from the cooling coil into a second container which is provided with a plurality of connected compartments at a uniform oxidizing temperature, introducing air into, and separating the residual air and volatile products from, each compartment, then passing the oxidized oil from the second container through a second cooling coil to extract the heat of the oxidizing reaction in like manner as before, and then discharging the product continuously from the system.

An object of the invention is to provide a simple, efficient and economical process by which asphaltic oils or residuum may be continuously converted into oxidized asphaltic products, which will have a relatively high melting point, flash and at the same time will be ductile and flexible.

Another object of the invention is to provide a simple and efficient process for manufacturing oxidized asphaltic products in which the various characteristics of ductil-

ity, high melting point and flash, required by different branches of the individual art, may be controlled, separately or in combination with other asphaltic products made by distillation with steam or other methods known in the art.

Another object of the invention is to provide a continuous method or process by which asphaltic petroleum oil residuum may be uniformly oxidized to the required degree with a minimum consumption of time.

With the foregoing preliminary explanation the preferred embodiment of the invention will now be more fully explained by reference to the accompanying drawing.

In the drawing, 1 represents generally a pipe which leads to a source of petroleum oil supply not shown, the flow being controlled by valve 2. Pipe 1 is connected to container or oxidizing reaction chamber 17. Pipe 15, controlled by valve 12, is connected to pipe 1. The container 17 is stationed in the top of furnace 18. Furnace 18 is provided with burner 19 which leads to a source of fuel supply not shown. Pipe 5, controlled by valve 3, is connected to container 17 at the top and to pipe 8. Pipe 5 leads to a source of steam supply not shown. Pipe 6, controlled by valve 7, is connected to pipe 8 and leads to a source of air supply not shown. Pipe 8, controlled as to steam by valve 4, is connected to pipes 9. Pipes 9 are connected to the top of container 17. Pipes 10 are connected to pipes 9 ending in spray pipes 11. Pipe 13 is connected to pipes 14. Pipes 14 are connected to the top of container 17. Pipe 13 is connected to a cooler and receiver not shown. Container 17 is provided with baffle plates 34, thereby providing a series of connected compartments. Pipe 20 connects container 17 near the bottom to the inlet side of pump 21. Pipe 22, controlled by valve 25, connects the discharge side of pump 21 to cooling coil 28. Pipe 24, controlled by valve 23, is connected to pipe 22 and leads to a receiver not shown. Cooling coil 28 is stationed in cooling chamber 26. Chamber 26 is provided with doors 27, 29 and 31 by means of which air or other cooling fluid may be admitted into chamber 26 in any desired amounts. The chamber 26 is provided with outlet flues 36. The flues 36 are provided with fans 35. The fans 35 are operated by a power not shown connected to the pulley 41. Pulley 41 is connected to transmission shaft 39 which operates the aforesaid fans 35 by means of cog-wheels. Pipe 16, controlled by valves 30 and 49, connects cooling coil 28, container 17 and container 17'. Container 17' is stationed in the top of furnace 18'. Furnace 18' is provided with a burner 19' which leads to a fuel supply not shown. Pipe 54, controlled by valve 53, connects pipe 16 to a source of petroleum oil supply not shown. Pipe 55, controlled by valve 52, con-

nects pipe 16 to a receiver not shown. Pipe 5', controlled by valve 3', is connected to container 17' near the top and leads to a source of steam supply not shown. Pipe 6', controlled by valve 7', connects pipe 8' to a source of air supply not shown. Pipe 8', controlled as to steam by valve 4', is connected to pipes 9'. Pipes 9' are connected to container 17' at the top. Pipes 10' connect pipes 9' to spray pipes 11'. The container 17' is provided with baffle plates 34'. Pipe 13' is connected to pipes 14'. Pipes 14' are connected to container 17' at the top. Pipe 13' is connected to a cooler and receiver not shown. Pipe 20' connects container 17' near the bottom to the inlet side of pump 21'. Pipe 22', controlled by valve 25', connects the discharge side of pump 21' to cooling coil 28'. Pipe 24', controlled by valve 23', is connected to pipe 22' and leads to a receiver not shown. Cooling coil 28' is stationed in cooling chamber 26'. Chamber 26' is provided with doors 27', 29' and 31' by means of which air or other cooling fluid may be admitted into chamber 26' in any desired amounts. The chamber 26' is provided with outlet flues 36'. The flues 36' are provided with fans 35'. The fans 35' are operated by a power not shown connected to the pulley 41'. Pulley 41' is connected to transmission shaft 39' which operates the aforesaid fans 35' by means of cog-wheels. Pipe 16' controlled by valve 57, connects cooling coil 28' to container 17'. Pipe 56, controlled by valve 58 connects pipe 16' to a cooler and receiver not shown.

The operation of the apparatus just described is preferably continuous but may be operated in batch lots.

The preferred operation of the apparatus just described is as follows:

Petroleum oil, or residuum, which may be derived from an asphalt or mixed base crude petroleum oil, is charged into the container or oxidizing reaction chamber 17 to any desired level by opening valve 2 in the pipe 1, the pipe 1 coming from a source of supply not shown. When container 17 has been filled to the desired level, valve 2 is tentatively closed and the residuum in container 17 is heated to the required oxidizing temperature by burner 19 in the furnace 18, this temperature ranging from approximately 400 to 550 degrees F., the degree of heat depending upon the petroleum oil to be oxidized and the product desired.

During this preliminary heating operation, the residuum is preferably circulated through cooling coil 28 and in order to prevent heat loss, having the doors 31, 27 and 29 in the chamber 26 closed, and the fans 35 in flues 36, not in operation. In this preliminary circulating and heating operation, the residuum passes through the compartments in oxidizing container 17, out near the bot-

tom of oxidizing container 17 into pipe 20 and then into the inlet side of pump 21 which discharges the same through pipe 22, cooling coil 28, pipe 16 and back into the container 17. It is desirable during this preliminary heating operation to introduce regulated quantities of air into the compartments of the oxidizing container 17, which are carried out by opening valve 7 in the air pipe 6 to the required degree, which permits air in sufficient amounts to pass from pipe 6 into pipe 8. Pipe 8 is connected to branch pipes 9 which conduct the air to the bottom of the compartments in oxidizing container 17 through branch pipes 10 which are connected to branch pipes 9 ending in spray pipes 11. If desired, steam may be introduced into the oxidizing container 17 along with air during this preliminary heating operation. The introduction of air, or steam and air during the preliminary heating operation is carried out in case the residuum to be oxidized contains small percentages of water or volatile hydrocarbons, to free the same of these constituents before the residuum has reached a rapid oxidizing temperature. The introduction of steam into oxidizing container 17 is carried out by a regulated opening of valve 4 in the pipe 8, which is connected to pipe 5.

During this preliminary heating operation of the residuum in oxidizing container 17, as well as during the oxidizing operation itself, a small amount of steam is preferably introduced into the top of oxidizing containers 17 and 17' through steam pipes 5 and 5' by regulated openings of valves 3 and 3' to prevent explosive or burning mixtures of air and volatile oil products from forming in the top of containers 17 and 17'.

As soon as the residuum circulating through the compartments of oxidizing container 17, cooling coil 28 and back into the container 17 has attained a sufficient oxidizing temperature (400 to 550 degrees F.), valve 49 is opened, valve 30 is closed, and valve 2 is opened to such a degree as to admit a regulated flow of the residuum to be oxidized in quantities sufficient to maintain a definite level in container 17, the rate of flow being governed by the rate of oxidation. At the same time the doors 31, 27 and 29 are opened to such a degree as to admit a sufficient quantity of cool air to extract the excess heat of the oxidizing reaction and maintain a substantially uniform oxidizing temperature required for the grade of stock to be made. The quantity of air passing through cooling chamber 26 is regulated by operation of fans 35 at such a speed that the cool air passing around the coil 28 will be sufficient to extract the excess heat produced by the oxidizing reaction. The partially oxidized residuum, from which the heat of the oxidizing reaction has been extracted, passes in a

continuous regulated stream flow from cooling coil 28 into pipe 16 and then into the second oxidizing container 17'.

This second oxidizing container 17' is constructed similar to container 17, having a plurality of connected compartments separated by baffle plates 34' and with individual air inlet pipes 10' ending in spray pipes 11' at the bottom of each compartment. The branch pipes 10' are connected to branch pipes 9'. The branch pipes 9' are connected to pipe 8'. Pipe 8' is connected to air pipe 6', the flow of air being controlled by valve 7'. Pipe 8' is also connected to steam pipe 5', the flow of steam being controlled by valve 4'.

During the oxidizing operation as well as during the preliminary heating, the quantity of air introduced into the compartments of oxidizing containers 17 and 17' may be varied, depending upon the stock under treatment and the product desired. Preferably approximately 1400 cubic feet of air per minute is employed for each 600 barrels of residuum under treatment.

The air passing through pipes 10 and 10' and out through the spray pipes 11 and 11' into the compartments of oxidizing containers 17 and 17' is usually equally proportioned, although equally proportioned amounts of air are not necessarily essential for each compartment, and in some cases more air may be introduced into the compartments of the second oxidizing container to obtain the required oxidation.

The partly oxidized flow of residuum passes through the compartments in container 17' and is therein oxidized to the required degree.

Some air, volatile oil and gaseous products of the oxidizing reaction pass out of the various compartments of oxidizing containers 17 and 17' through pipes 14 and 14' into pipes 13 and 13' and then through condensers not shown, wherein the condensable hydrocarbons are liquefied and may be used for other purposes.

From the last compartment in container 17' the flow of oxidized residuum passes out of container 17' through pipe 20' and into the inlet side of pump 21'. Pump 21' discharges the oxidized residuum through pipe 22', cooling coil 28' and into pipe 16'. The oxidized residuum passing through cooling coil 28' is cooled to the required degree by the introduction of air or other cooling fluid coming through the doors 31', 27' and 29'. The quantity of air passing through cooling chamber 26' is regulated by operation of fans 35' at such a speed that the cool air passing around the coil 28' will be sufficient to lower the temperature of the oxidized residuum below its flash point. From pipe 16' the cooled oxidized residuum passes out of the system through pipe 56 and into a

storage not shown, valve 57 being closed and valve 58 being open; or a part of the oxidized residuum may be continuously discharged from the system through the pipe 24' to a storage not shown by a regulated opening of valve 23'. If desired, a portion or all of the flow of residuum under oxidation may be returned to container 17 through pipes 24, 55 or 24', by pipe connections not shown to pipe 15, controlled by the valves 23, 52, 23' and 12; or a portion or all of the flow of residuum may be returned to container 17' through pipe 24' by a pipe connection not shown to pipe 54.

15 The operation of this invention may be carried out under superatmospheric pressure or under pressures less than atmospheric, depending upon the petroleum oil residuum to be treated and the product desired. For 20 example, in the manufacture of high melting point oxidized asphalt from a petroleum oil or petroleum oil residuum containing a high percentage of relatively low boiling hydrocarbons, the oxidizing operation as heretofore described may be conducted under vacuum ranging from 755 to 5 mm. of mercury or less, absolute pressure, and in the production of oxidized asphaltic products from low Baumé gravity petroleum residuum, which 25 contains substantially no relatively low boiling hydrocarbons, other oxidizing operations may be conducted at atmospheric pressure or at pressures of 1000 pounds or more.

30 While the process herein described is well 35 adapted for carrying out the objects of the present invention, it is to be understood that various modifications and changes may be made without departing from the spirit of the invention, such for example, as the employment of three or more oxidizing containers and cooling coils, also the employment of water or other fluids as cooling mediums to extract the heat produced by the oxidizing reaction, and the invention includes all such 40 45 changes and modifications as come within the scope of the appended claims.

What I claim is:

1. A process of oxidizing asphaltic oils, comprising, maintaining a supply of asphaltic oil in a plurality of containers, each container being provided with a plurality of connected compartments through which the asphaltic oil continually passes, at an elevated oxidizing temperature produced by the application of heat to each container and heat produced by an oxidizing reaction, continuously passing regulated streams of air through the supply of asphaltic oil in each container, continuously withdrawing the residual air and volatile oil products from each container, continuously introducing a regulated stream of asphaltic oil into the first compartment of the first container, continuously passing the oil from each container, from which the residual air and volatile

oil products have been separated, into separate cooling coils to extract the exothermic heat of the oxidizing reaction, continuously introducing the oil from the interstage cooling coil into the succeeding container and then into a final cooling coil and discharging the oxidized asphaltic oil from the system. 70

2. A process of oxidizing asphaltic oils, comprising, maintaining a supply of asphaltic oil in a plurality of containers, each container being provided with a plurality of connected compartments through which the asphaltic oil continuously passes in contact with introduced air, at an elevated oxidizing temperature, substantially below a cracking temperature, produced by the application of heat to each container and heat produced by an oxidizing reaction, continuously introducing a regulated stream of asphaltic oil into the first compartment of the primary container, 80 continuously passing regulated streams of air and steam through the supply of asphaltic oil passing through each container, continuously withdrawing the residual air, steam and volatile oil products from each container, continuously passing the oil from each container, from which the residual air, steam and volatile oil products have been separated, into separate cooling coils to extract the exothermic heat of the oxidizing reaction, 85 continuously introducing the oil from the interstage cooling coil into the succeeding container and then into a final cooling coil and discharging the oxidized asphaltic oil from the system. 90

3. A process of oxidizing asphaltic oils, comprising, maintaining a supply of asphaltic oil in a plurality of containers, each container being provided with a plurality of connected compartments through which the asphaltic oil continually passes in contact with air, at a temperature of approximately 400 to 550 degrees F. produced by the application of heat to each container and heat produced by an oxidizing reaction, continuously introducing a regulated stream of asphaltic oil into the first compartment of the first container, continuously passing regulated streams of air through the supply of asphaltic oil passing through the compartments of each container, continuously withdrawing the residual air and volatile oil products from each container, continuously passing the oil from each container, from which the residual air and volatile oil products have been separated, into separate cooling coils to extract the exothermic heat of the oxidizing reaction, continuously passing the oil from the interstage cooling coil through the succeeding container and then into a final cooling coil and discharging the oxidized asphaltic oil from the system. 100 105 110 115 120

4. A process of oxidizing asphaltic oils, comprising, maintaining a supply of asphaltic oil in a plurality of containers at an ele- 125 130

vated oxidizing temperature, substantially below a cracking temperature, by the application of heat to each container and heat produced by an oxidizing reaction, continuously 5 introducing a regulated stream of asphaltic oil into the first container, passing air and steam and air intermittently through the supply of asphaltic oil in each container, continuously withdrawing the residual air, air and 10 steam and volatile oil products from each container, continuously passing the oil from each container, from which the residual air, steam and volatile oil products have been separated, into separate cooling coils to extract the exo- 15 thermic heat of the oxidizing reaction, continuously passing the oil from the interstage cooling coil into the first compartment of the succeeding container and from the last compartment of the last container into a final 20 cooling coil, and discharging the oxidized asphaltic oil from the system.

5. A process of oxidizing asphaltic oils, comprising, maintaining a supply of asphaltic oil in a plurality of containers, each container being provided with a plurality of connected compartments through which the asphaltic oil continuously passes, at a temperature not greater than 550 degrees F. by the application of heat to each container and heat produced by an oxidizing reaction, continuously introducing a regulated stream of asphaltic oil into the first container, continuously passing regulated streams of air through the supply of asphaltic oil in each container to oxidize the asphaltic oil, continuously withdrawing the residual air and volatile oil products from each container, continuously passing the oil from each container, from which the residual air and volatile products have been separated, into separate cooling coils and extracting the exothermic heat of the oxidizing reaction, continuously passing the oil from the interstage cooling coil into the succeeding container and then into a final cooling coil and discharging the oxidized asphaltic oil from the system.

50 6. A process of producing oxidized asphalt, comprising continuously introducing and passing petroleum oil residuum through a series of connected compartments in a container holding a bulk supply of petroleum oil residuum, maintaining the bulk supply of petroleum oil residuum at an elevated oxidizing temperature produced by the application of heat to the container and heat produced by an oxidizing reaction, passing separately regulated streams of air through the petroleum oil residuum in each compartment of the container, continuously separating the residual air and volatile oil products from the residuum undergoing oxidation, continuously extracting from the residuum the excess exothermic heat produced by the oxidizing reaction by passing the same through a cooling coil in heat exchange relationship with a cool-

ing medium, passing the partly oxidized residuum through a second series of connected compartments in a second container, maintained substantially at the oxidizing temperature of the first mentioned container, passing separately regulated streams of air through the residuum contained in each compartment of the second container, continuously separating the residual air and volatile oil products from the residuum undergoing oxidation in each compartment of the second container, continuously extracting from the residuum the excess exothermic heat produced by the oxidizing reaction by passing the same through a second cooling coil in heat exchange relationship with a cooling medium, maintaining the temperature and time so that the residuum within said containers will be oxidized to the required degree and then passing the oxidized residuum out of the system.

7. A process of forming oxidized asphalt, comprising, passing petroleum oil residuum in a regulated stream flow through a series of connected compartments in a container holding a bulk supply of petroleum oil residuum, maintaining the bulk supply of petroleum oil residuum at a temperature of approximately 400 to 550 degrees F. by application of heat to the container and heat produced by an oxidizing reaction, passing separately regulated streams of air through the petroleum oil residuum contained in each compartment in the container, continuously separating the residual air and volatile oil products from the residuum undergoing oxidation in each compartment of said container, continuously extracting from the residuum the excess exothermic heat produced by the oxidizing reaction by passing the same through a cooling coil in heat exchange relationship with a cooling medium, then passing the partly oxidized residuum through a second series of connected compartments in a second container, maintained at substantially the same oxidizing temperature of the first mentioned container, passing separately regulated streams of air through each compartment of the second container, continuously separating the residual air and volatile oil products from the residuum undergoing oxidation in each compartment of the second container, continuously extracting the excess exothermic heat produced by the oxidizing reaction from the residuum by passing the residuum from the last compartment of the second container through a second cooling coil in heat exchange relationship with a cooling medium, maintaining temperature and time so that the residuum within said containers will be oxidized to the required degree and continuously passing the oxidized residuum out of the system.

8. A process of forming oxidized asphalt, comprising, passing a regulated flow of petroleum oil residuum through a series of

connected compartments in a container holding a bulk supply of petroleum oil residuum, maintaining the bulk supply of petroleum oil residuum at an elevated oxidizing temperature produced by the application of heat to the container and heat produced by an oxidizing reaction passing separately regulated streams of air and steam through each compartment of the container, continuously separating the residual air, steam and volatile oil products from the residuum undergoing oxidation in each compartment of said container, continuously extracting from the residuum the excess exothermic heat produced by the oxidizing reaction by passing the residuum through a cooling coil in heat exchange relationship with a cooling medium, passing the partly oxidized residuum through a second series of connected compartments in a second container, passing separately regulated streams of air and steam through each compartment of the second container, continuously separating the residual air, steam and volatile oil products from the residuum undergoing oxidation in each compartment of the said second container, continuously cooling the residuum after passing through the second container, by passing the same through a second cooling coil in heat exchange relationship with a cooling medium, and discharging the finished oxidized product from the system.

9. A process of oxidizing asphaltic oils, comprising, maintaining a supply of asphaltic oil in a plurality of containers at an elevated oxidizing temperature by the application of heat to each container and heat produced by an oxidizing reaction, continuously introducing a regulated supply of asphaltic oil into the first container, continuously passing regulated streams of air and steam through the supply of asphaltic oil in each container, continuously withdrawing the residual air, steam and volatile oil products from each container, continuously passing the oil from each container, from which the residual air, steam and volatile oil products have been separated, into separate cooling coils to extract the exothermic heat of the oxidizing reaction, continuously introducing the oil from the interstage cooling coil into the succeeding container and then into a final cooling coil, and discharging the finished product from the system.

55 In testimony whereof I affix my signature.  
TOM H. DOWLEN.